

Aug. 25, 1953

J. GOLDSTEIN

2,650,169

PHOSPHORESCENT COATED SHEET MATERIAL

Filed Sept. 28, 1949



FIG. 1

FIG. 2



FIG. 3

INVENTOR.

Joseph Goldstein  
BY

Eugene M. Goldstein  
his attorney.

Patented Aug. 25, 1953

2,650,169

# UNITED STATES PATENT OFFICE

2,650,169

## PHOSPHORESCENT COATED SHEET MATERIAL

Joseph Goldstein, Brookline, Mass.

Application September 28, 1949, Serial No. 118,325

6 Claims. (Cl. 117—33.5)

1

The present invention is an improvement in phosphorescent coated textiles and fabrics and in particular to the application of such fabrics and plastics to slippers and shoes.

In my prior issued Patent No. 2,473,877, there is described phosphorescent material of activated metallic solids, such as zinc sulphide or sulphides of calcium, strontium, cadmium, barium or the like, to which colored pigment may be added. These materials which may also include other phosphorescent crystals such as magnesium sulphide and other materials such as aniline dyes or other coloring pigments are suspended in a lacquer or liquid vehicle using resins or synthetic resins, such for instance as cellulose acetate, vinyl chloride, vinyl chloride-acetate, methyl-methacrylate melamine, or any of the other numerous thermoplastics or thermosetting resins, to which such phosphorescent material may be added without chemical changes.

An essential for practical use of phosphorescent materials is an after-glow for a long period of time, with an intensity sufficient to be readily visible without too great difficulty for the entire period.

In addition to this the fabric, textile, molded or synthetic fibrous resinous plastic or composition sheet, for greatest utility should be able to stand up under any rough wear showing no appreciable deterioration of the phosphorescent after-glow because of continued use of the objects to which the material is applied.

The present invention is particularly directed to the production of a coated textile or fabric sheet having such phosphorescent properties that a sufficiently intense after-glow is maintained for a period of from six to eight hours, sufficient to permit the material to be readily visible with no more than the usual adjustment for dark conditions and to a sheet which will not deteriorate during the wearing of the sheet throughout its life. In use on or in slippers no eye adjustment is needed since usually a person wakes up in the dark to look for his slippers and his eyes are already adjusted.

In accordance with the present invention, the fabric or textile is given a base coat with a paint or lacquer which provides a pure white reflecting surface to make a uniform background and give maximum light reflecting properties and also seal and waterproof pores of fabric so that no moisture will penetrate through the bottom of the sheet. White pigment, such as lithopone, titanium dioxide or other suitable white pigment may be used. Upon this base coating is applied a

phosphorescent coating of  $2\frac{1}{2}$  oz. to 6 oz. per sq. yard suitably pigmented with phosphorescent crystals and over the phosphorescent coating there is applied a third protective coating which seals the top surface of the phosphorescent crystals as a protection against deterioration, all of which will be pointed out later.

The vehicles of all three coatings must of course be compatible with one another.

10 I have discovered that a maximum critical phosphorescent response intensity enduring for a long period of time may be obtained by a phosphorescent coating made up of phosphorescent crystal pigments composed of definite quantities of various types of combined calcium sulphide and strontium sulphide crystals as will be explained later. Such phosphorescent pigment combination produces a fluorescent color between the green and blue lines of the spectrum, tending more to the green lines or the longer light wave lengths rather than to the shorter and ultra wave length light. Such phosphorescent pigments may be reactivated by exposure to "black" light, "white" light, day-light or artificial light.

20 15 25 While phosphorescent pigments of the type used in the present invention actually continue to glow for a considerable number of hours, from ten to seventy-five hours, the decay is exponentially so that only a smaller portion of the time above stated provides actually visible luminescence.

30 35 40 It has been found that for most practical purposes, visible luminescence for six to eight hours is quite satisfactory for the purpose of the present invention, and this is obtained in the phosphorescent sheet of the present invention. The sheet of the present invention finds particular application in shoes and slippers where a piece having the general form of an inner sole on reduced proportions is applied to the instep of the shoe by sewing, cementing or some other means, the piece being such as to show the right and left shoe and also where the foot is to be inserted in accordance with my prior patent above mentioned.

45 50 Without further describing the merits and advantages of the present invention, the invention will be described in the specification below in connection with the drawings annexed hereto; in which:

Figure 1 shows the invention applied to a pair of slippers.

Figure 2 shows a section taken through a portion of the inner sole along the line 2—2 of Figure 1, and

3

Figure 3 shows a set of curves relating to the combination of phosphorescent pigments used in the phosphorescent sheet.

As indicated in Figures 1 and 2, small sheets 1 and 2 in the form of a right and left inner-sole are stitched by over-cast stitching 3, or by any other type of stitching or cemented in the region of the center of the instep, running longitudinally with the shoe, the one in the right shoe being in the shape of the right instep and the one in the left shoe being in the shape of the left instep. These insert sheets are covered over their entire surface with a phosphorescent coating which will be described below.

As has been previously set forth, the sheets 15 have three coatings applied thereto, a base coat over which the phosphorescent coating is applied, and lastly the protective coating. The base coating should be a white primer in a paint or lacquer with which the other coats are compatible. A 20 coating suitable for this purpose may be made of vinyl chloride-acetate resin dissolved in a suitable liquid, such as methyl-ethyl ketone in a concentration between 20% and 30% with suitable amounts of plasticizer, white reflecting pigments, such as titanium dioxide, filler, stabilizers with a small amount of stearic acid to deter settling and serve as a lubricant. A specific base 25 coat formula on the basis of approximately one-hundred pounds may comprise the following:

60-70 lbs. vinyl chloride-acetate resins of a concentration of 20 to 30% in methyl-ethyl ketone  
4-6 lbs. aryl alkyl-phosphate  
4-6 lbs. plasticizer, such as di-2-ethylhexyl phthalate.

13-17 lbs. white pigment which might be a combination of titanium dioxide and natural water ground calcium carbonate or other inert highly reflecting material nonsoluble in the vehicle  
5-8 lbs. other materials such as suspensoids, wet dispersed stabilizers, thinners, etc.

The formula above may of course be varied depending upon the desired viscosity of the liquid and its uniformity.

The coating as applied should give a pure white sheen, providing a uniform reflecting surface with a minimum amount of light absorption. After this coat has been applied and left to dry, the phosphorescent coating may be applied. The base 50 coat using one-hundred pounds as set forth above, will cover approximately one-hundred linear yards, 38 or 39 inches wide.

The phosphorescent coating should be approximately of the same thickness and should use the same vehicle for the phosphorescent pigment.

On the basis of approximately one hundred pounds, this may comprise:

65-75 lbs. 20%-30% vinyl chloride-acetate resin solution  
6-7 lbs. plasticizer  
2-2.5 lbs. titanium dioxide  
3.5-2.5 lbs. aluminum stearate  
18.8-19.3 lbs. phosphorescent pigment

This formula may be approximately varied over a 10% range but for best results the phosphorescent pigment used must be sufficient to provide a uniformly covered surface without voids of crystals. The aluminum stearate serves to prevent 70 the settling of the heavier phosphorescent pigment in the coating, so that the phosphorescent pigment will remain uniformly throughout the coating as the coating dries and prevents the pigment from settling to the bottom of the coating, 75

in which case it would have to shine through the entire thickness of the coating. The top coating should be as clear as possible and serve only to provide a protective surface through which light would efficiently pass. This coating may also be of the same general thickness as the other two coats and comprise the following on the basis of one-hundred pounds:

87 lbs. 20% vinyl chloride-acetate resins  
13 lbs. A-100 acryloid (40% solid), plus a very small amount of wet dispersed stabilizer, which amount may be compensated by decreasing the amount of vinyl chloride-acetate resin to make up the one-hundred pound formula

It will be noted that in each of the three coatings, the basic substance of largest proportions is the vinyl chloride-acetate resin, which provides uniformity for all three coatings, thereby insuring uniform reflecting properties of light between successive layers of coatings. The formulas for each coating may also be made up of other resins, such as vinyl-acetate resins, cellulose nitrate and acetate resins, melamine resins, urea-formaldehyde resins and many others.

With regard to the phosphorescent pigments, I have determined by experiments, that by mixing phosphorescent pigments formed of calcium and strontium sulphides and strontium and calcium sulphides in certain definite proportions, particularly desirable phosphorescent pigments may be obtained, in that its after-glow intensity will be maintained above the ordinary visible limits for a substantially longer period of time than when one or the other pigments are used separately. This is shown in the curves of Figure 3, where A represents crystal pigment formed with CaS 15% and SrS 85% and curve B represents crystal pigments formed with CaS 92% and SrS 8%. These percentages have fairly close tolerances but the material in curve A may be varied approximately 1% and so also the materials of curve B.

In Figure 3, the abscissa axis is shown logarithmically as a time axis in logarithms to the base 10 and phosphorescent intensity is shown as the ordinate in the ordinary scale.

The straight line C indicates an average minimum permissible intensity below which it is difficult for the ordinary eye to see readily the phosphorescent material in the dark. When the intensity drops below this line, the phosphorescent material is not very efficient. The curve D shows a combination mixture of 50% of each of the pigments of A and B. This curve D, while it starts with no greater intensity than the curves A and B, nevertheless it maintains a higher intensity than the other two curves above the minimum line C for a longer period, after which it tends to diminish more rapidly. The result is that in combinations of approximately 50% of each of the pigments of A and B, a maximum desirable response is obtained providing a desired after-glow, which under ordinary conditions will endure for about 500 minutes. The phosphorescent coat therefore contains approximately 50% of each of these pigments. Pigments of this type are manufactured commercially and readily obtainable.

The coatings as produced by the present invention when used for slippers in the manner described will keep the slippers luminous by night, and need only be activated for less than a very few minutes, as for instance, at the time the individual is going to bed. If the slippers are exposed

for a very few minutes before the lights are turned out, the phosphorescent patch will remain visible all night and permit, as stated above, the individual to put the slippers on with the least amount of difficulty without turning on the light. 5

I claim:

1. A sheet having a phosphorescent coating having phosphorescent crystal pigments composed of substantially 50% crystals having calcium and strontium sulphides in the ratio of 15 10 and 85 percent respectively, and 50% crystals having strontium and calcium sulphides in the ratio of 8 and 92% respectively.

2. A sheet having a phosphorescent coating as set forth in claim 1, in which the phosphorescent 15 crystals are dispersed in a liquid comprising principally a synthetic resin dissolved in methyl-ethyl ketone.

3. A sheet having a phosphorescent coating as set forth in claim 2, in which the synthetic resin 20 is a vinyl chloride-acetate resin in approximately a 20% concentration in methyl-ethyl ketone.

4. A sheet having a phosphorescent coating having phosphorescent crystal pigments composed of substantially 50 per cent crystals having 25 calcium and strontium sulphides in the ratio of 15 and 85 per cent respectively, and 50 per cent crystals having strontium and calcium sulphides in the ratio of 8 per cent and 92 per cent respectively, and having quantities of titanium dioxide 30 and aluminum stearate in the ratio of 2½ and 3 percent respectively, of the liquid weight of the phosphorescent coating.

5. A sheet having a phosphorescent coating applied to said sheet in a liquid state, said liquid comprising a composition as follows:

65-75 lbs. 20% to 30% solid content vinylchloride-acetate resin solution

6-7 lbs. plasticizer

2-2.5 lbs. titanium dioxide

3.5-2.5 lbs aluminum stearate

18.8-19.3 lbs. phosphorescent inorganic pigment crystals

6. A sheet as set forth in claim 5 in which the amounts may vary in a range of 10%.

JOSEPH GOLDSTEIN.

References Cited in the file of this patent  
UNITED STATES PATENTS

| Number    | Name         | Date          |
|-----------|--------------|---------------|
| 1,188,655 | Hewitt       | June 27, 1916 |
| 1,291,739 | Booth        | Jan. 21, 1919 |
| 1,321,024 | Frank        | Nov. 4, 1919  |
| 1,349,396 | Van Cliff    | Aug. 10, 1920 |
| 1,467,132 | Bilstein     | Sept. 4, 1923 |
| 1,630,730 | Daugherty    | May 31, 1927  |
| 2,039,734 | Meder et al. | May 5, 1936   |
| 2,290,690 | Lehman       | July 21, 1942 |
| 2,310,740 | Leavy        | Feb. 9, 1943  |
| 2,341,009 | Axelrad      | Feb. 8, 1944  |
| 2,413,459 | Lynch        | Dec. 31, 1946 |
| 2,473,877 | Goldstein    | June 21, 1949 |
| 2,498,592 | Switzer      | Feb. 21, 1950 |